

Nov. 27, 1934.

A. L. MINGARD

1,982,012

PROCESS FOR MANUFACTURING HARD OBJECTS IN SILICIDIZED  
CARBON OR OTHER SIMILAR SUBSTANCES

Filed April 20, 1932



INVENTOR

Aurèle Louis Mingard

BY

Samuel Smith

ATTORNEY

## UNITED STATES PATENT OFFICE

1,982,012

PROCESS FOR MANUFACTURING HARD  
OBJECTS IN SILICIDIZED CARBON OR  
OTHER SIMILAR SUBSTANCES

Aurèle Louis Mingard, Lausanne, Switzerland

Application April 20, 1932, Serial No. 606,490  
In France May 11, 1931

1 Claim. (Cl. 51—278)

The object of this invention is a process for manufacturing very hard objects, particularly grinding stones, in silicidized carbon or other very hard materials.

The process consists essentially in transforming objects of any shape, made of carbon, into another very hard substance particularly into silicidized carbon, without altering their shape and by chemical reaction at high temperature. The crucible in which the reactions take place is filled with a mixture of substances capable of reacting upon each other at the temperature produced by an electric arc struck between electrodes. By the influence of this arc and as a result of the chemical reactions between the substances forming the charge, metallic vapors are produced, which reach a certain pressure, forming a pocket with the arc in the center, and which pocket gradually increases in volume until the objects to be transformed, and which at the commencement of the operation were embedded in the charge, are enclosed within the pocket charged with metallic vapors, without having changed their position, and are subjected to the action of these vapors, until the transformation into a very hard material particularly silicidized carbon, is completed.

The transformation is preferably produced in a furnace consisting of a crucible 1 of any desired shape, containing a lining of refractory bricks. This furnace is placed either vertically or horizontally and may be of the tilting type. It is provided with electrodes 2 of carbon or other material capable of resisting high temperatures. These electrodes may be placed into the furnace in any position with respect to the furnace, and at any variable position with regard to each other. They can, for instance, be placed along the center line of the furnace in line with each other and at any distance from each other. Each electrode is fitted on the end inside the furnace with a piece of carbon 3 of any suitable shape, cylindrical, coneshaped etc. The object or objects of carbon 4 to be transformed are attached to the electrodes in any suitable manner, along their center line for instance if they are cylindrical. The other electrode may also be provided with a similar object or an object of different shape to the one attached to the first electrode. In the case of a body of carbon in the form of a grinding wheel, the body may be mounted on the electrode by means of the axial bore formed therein. When so mounted the body is held in place on the electrode by friction between the bore in the body and the electrode.

The electrodes are fixed in a suitable way and maintained in a vertical or any other position, along the center line of the hollow cylinder forming the furnace. If this furnace is used exclusively in a vertical position, the lower part is closed, thus forming a crucible through the bottom of which the lower electrode only passes through an aperture.

The transformation of the objects made of carbon, into silicidized carbon or other material proceeds in the following manner.

The furnace is charged with a mixture of substances capable of producing by chemical reaction at high temperature the transformation of the objects of carbon into silicidized carbon or other very hard substances.

As an example of such substances forming the charge the following mixture is mentioned:

For obtaining silicidized carbon:

|             | Parts |
|-------------|-------|
| Silica..... | 30    |
| Carbon..... | 7     |

The proportions of materials employed as stated, have no limitative character and may vary within wide limits.

A continuous or alternating electric current is then sent through the electrodes by means of electric conduits in metal or other conductive material, to which conduits the electrodes are attached in any suitable manner, along their axis for instance.

The arc is struck between the electrodes and as a result of the heat produced a chemical reaction takes place between the substances forming the charge in the furnace, liberating from one of the constituents silicon vapors, or other vapors according to the nature of the charge.

This reaction may be represented as follows:



95

These vapors reach a certain pressure and rapidly form around the arc a pocket 5 with the arc in the center. The pocket gradually increases in volume until the objects of carbon which it is desired to transform are enclosed within this pocket. These objects are then subjected to the action of metallic vapors of silicon or other elements and are transformed into silicidized carbon or as the case may be into other very hard materials with carbon as a base, without changing in shape or position in the furnace and without passing through any other physical changes. The objects may then be removed from the furnace and the operation can be repeated.

110

I claim:

A method of producing grinding wheels comprising positioning a wheel formed of carbon on one of a pair of electrodes, surrounding the electrodes and carbon wheel with a charge of silica and carbon, electrically energizing the electrodes and striking an arc between them, maintaining the vapor phase products of conversion formed

by heat supplied to the charge from the arc in a pocket formed in the charge about the arc, and continuing the arc until the pocket has increased due to conversion of the charge into vapor phase products to a size sufficient to include the carbon wheel and thereby subject the wheel to the silicidizing action of silicon vapor in the pocket.

AURELÉ LOUIS MINGARD.

10

15

20

25

30

35

40

45

50

55

60

65

70

75

1

10

10

11

11

12

12

13

13

14

14

15